

[54] **INTERMETALLIC COMPOUND MATERIALS**

[75] Inventors: **James Edward Restall, Camberley; Michael James Douglas Weaver, Fleet, both of England**

[73] Assignee: **National Research Development Corporation, London, England**

[22] Filed: **May 23, 1972**

[21] Appl. No.: **256,026**

[30] **Foreign Application Priority Data**

May 26, 1971 United Kingdom..... 17150/71

[52] U.S. Cl. .... **75/171; 75/170; 148/32**

[51] Int. Cl. .... **C22c 19/00**

[58] Field of Search ..... **75/170, 171; 148/32, 32.5**

[56] **References Cited**

UNITED STATES PATENTS

|           |         |                 |        |
|-----------|---------|-----------------|--------|
| 3,617,397 | 11/1971 | Maxwell.....    | 75/170 |
| 3,653,987 | 4/1972  | Boesch.....     | 75/171 |
| 3,677,835 | 7/1972  | Tien et al..... | 75/171 |
| 3,767,479 | 10/1973 | Tarshis.....    | 75/171 |

*Primary Examiner*—R. Dean

*Attorney, Agent, or Firm*—Cushman, Darby & Cushman

[57] **ABSTRACT**

An intermetallic compound material, which may be produced by standard vacuum melting techniques, comprises two principal groups of constituents of which a first group includes nickel and at least one of the elements chromium, cobalt, molybdenum and tungsten within the range 72 to 83 atomic per cent, and the second group includes aluminium in combination with at least one of the elements titanium, niobium and tantalum, the material containing the constituents in the proportions, by atomic percentage,

first group of constituents 72 to 83

second group of constituents 17 to 28

One preferred composition of the intermetallic compound material contains elements of the said first and second groups in the following ranges specified below, in atomic per cent,

|            |          |           |          |
|------------|----------|-----------|----------|
| Nickel     | 60 to 80 | Aluminium | 12 to 26 |
| Chromium   | 2 to 6   | Titanium  | 0 to 12  |
| Cobalt     | 0 to 12  | Niobium   | 0 to 6   |
| Molybdenum | 0 to 3   | Tantalum  | 0 to 6   |
| Tungsten   | 0 to 3   |           |          |

The intermetallic compound material may contain carbon, boron, and zirconium as trace elements.

**10 Claims, No Drawings**

## INTERMETALLIC COMPOUND MATERIALS

This invention relates to intermetallic compound materials and in particular to metal alloys having a base of tri-nickel aluminide ( $Ni_3Al$ ).

The majority of high temperature structural components currently used in gas turbine aero engines are made from nickel-base alloys strengthened primarily by the precipitation of  $Ni_3Al$  (gamma-prime) throughout the nickel (gamma) matrix. During recent years, the strengths of such alloys have been improved by increasing the stability and volume fraction of the gamma-prime precipitate through the introduction of relatively large quantities of elements such as tungsten, molybdenum, tantalum, niobium and titanium. This has involved reduction of the nickel and chromium content,

melt is fully degassed, chromium and any refractory metals are added under a partial pressure of argon. Aluminum, titanium and zirconium are then added under vacuum and the metal cast into ingot form. Conventional casting techniques have produced materials having acceptable high temperature strengths and ductilities. Unidirectional solidification in which a temperature gradient is induced by progressive cooling in order to control crystalline growth to give a columnar structure has been found to give increased strength and ductility.

The accompanying Table I gives the compositions of several examples of intermetallic compound materials according to the invention. These compositions are representative of those believed to give good combinations of desirable properties, but are not intended to be exclusive.

TABLE I

| Alloy Code | Alloy compositions |      |      |     |     |         |      |     |     |      |      |      |
|------------|--------------------|------|------|-----|-----|---------|------|-----|-----|------|------|------|
|            | Group A            |      |      |     |     | Group B |      |     |     |      |      |      |
|            | Cr                 | Co   | Ni   | Mo  | W   | Al      | Ti   | Nb  | Ta  | C    | B    | Zr   |
| R1         | 3.7                | 6.9  | 64.7 | 1.3 | —   | 17.2    | 5.9  | —   | —   | 0.2  | 0.05 | 0.05 |
| R3         | 3.3                | 7.1  | 64.2 | 0.8 | 0.4 | 19.0    | 2.3  | 1.3 | 1.3 | 0.2  | 0.05 | 0.05 |
| R6         | 3.2                | 7.3  | 62.8 | 0.7 | 0.4 | 20.2    | 1.1  | 2.1 | 1.9 | 0.2  | 0.05 | 0.05 |
| R9         | 3.4                | 7.2  | 64.5 | 0.7 | 0.5 | 18.0    | 3.7  | 0.8 | 0.9 | 0.2  | 0.05 | 0.05 |
| A33        | 5.1                | 7.9  | 61.5 | —   | 1.8 | 19.9    | —    | —   | 3.5 | 0.2  | 0.05 | 0.05 |
| A53        | 2.8                | 6.5  | 62.9 | 1.0 | —   | 21.1    | —    | —   | 5.4 | 0.2  | 0.05 | 0.05 |
| A60        | 3.2                | 6.8  | 64.8 | 1.1 | —   | 19.0    | —    | 4.8 | —   | 0.2  | 0.05 | 0.05 |
| A92        | 4.0                | 10.5 | 60.7 | 0.1 | —   | 13.7    | 10.7 | —   | —   | 0.2  | 0.05 | 0.05 |
| A203       | 4.0                | —    | 71.6 | 1.1 | —   | 18.9    | 2.1  | 2.0 | —   | 0.2  | 0.05 | 0.05 |
| V197       | 3.9                | 7.1  | 64.6 | —   | 1.0 | 19.5    | —    | —   | 3.6 | 0.2  | 0.05 | 0.05 |
| V199       | 3.5                | 7.1  | 70.0 | —   | 0.9 | 16.5    | —    | —   | 3.6 | 0.25 | 0.10 | 0.05 |

the strength improvements thus being obtained at the expense of corrosion resistance. It is known that in addition to its precipitation strengthening role, the gamma-prime phase present in commercial precipitation-hardened nickel-base alloys has good corrosion resistance at high temperatures.

Binary  $Ni_3Al$  has little worthwhile high temperature strength and is fairly brittle but alloys based on  $Ni_3Al$  containing additional alloying elements can combine the high corrosion resistance of  $Ni_3Al$  with the strength and ductilities of modern precipitation-hardened nickel-base alloys at higher temperatures than the latter can withstand.

An intermetallic compound material according to the invention comprises two principal groups of constituents of which one group includes nickel and one or more of the elements chromium, cobalt, molybdenum and tungsten within the range 72 to 83 atomic per cent, and the second group includes aluminium and one or more of the elements titanium, niobium and tantalum within the range 17 to 28 atomic per cent.

Preferably the constituents are in the following ranges (specified in atomic per cent):

|            |          |           |          |
|------------|----------|-----------|----------|
| Nickel     | 60 to 80 | Aluminium | 12 to 26 |
| Chromium   | 2 to 6   | Titanium  | 0 to 12  |
| Cobalt     | 0 to 12  | Niobium   | 0 to 6   |
| Molybdenum | 0 to 3   | Tantalum  | 0 to 6   |
| Tungsten   | 0 to 3   |           |          |

Additional trace elements are 0.05 to 0.5 carbon, 0.01 to 0.1 boron, and 0.01 to 0.2 zirconium (all atomic percentages).

Intermetallic compound materials according to the invention can be produced by standard vacuum melting techniques. As a typical example, nickel, cobalt, carbon and boron are melted under vacuum and when the

melt is fully degassed, chromium and any refractory metals are added under a partial pressure of argon. Aluminum, titanium and zirconium are then added under vacuum and the metal cast into ingot form. Conventional casting techniques have produced materials having acceptable high temperature strengths and ductilities. Unidirectional solidification in which a temperature gradient is induced by progressive cooling in order to control crystalline growth to give a columnar structure has been found to give increased strength and ductility.

The accompanying Table I gives the compositions of several examples of intermetallic compound materials according to the invention. These compositions are representative of those believed to give good combinations of desirable properties, but are not intended to be exclusive.

TABLE I

| Alloy Code | Alloy compositions |      |      |     |     |         |      |     |     |      |      |      |
|------------|--------------------|------|------|-----|-----|---------|------|-----|-----|------|------|------|
|            | Group A            |      |      |     |     | Group B |      |     |     |      |      |      |
|            | Cr                 | Co   | Ni   | Mo  | W   | Al      | Ti   | Nb  | Ta  | C    | B    | Zr   |
| R1         | 3.7                | 6.9  | 64.7 | 1.3 | —   | 17.2    | 5.9  | —   | —   | 0.2  | 0.05 | 0.05 |
| R3         | 3.3                | 7.1  | 64.2 | 0.8 | 0.4 | 19.0    | 2.3  | 1.3 | 1.3 | 0.2  | 0.05 | 0.05 |
| R6         | 3.2                | 7.3  | 62.8 | 0.7 | 0.4 | 20.2    | 1.1  | 2.1 | 1.9 | 0.2  | 0.05 | 0.05 |
| R9         | 3.4                | 7.2  | 64.5 | 0.7 | 0.5 | 18.0    | 3.7  | 0.8 | 0.9 | 0.2  | 0.05 | 0.05 |
| A33        | 5.1                | 7.9  | 61.5 | —   | 1.8 | 19.9    | —    | —   | 3.5 | 0.2  | 0.05 | 0.05 |
| A53        | 2.8                | 6.5  | 62.9 | 1.0 | —   | 21.1    | —    | —   | 5.4 | 0.2  | 0.05 | 0.05 |
| A60        | 3.2                | 6.8  | 64.8 | 1.1 | —   | 19.0    | —    | 4.8 | —   | 0.2  | 0.05 | 0.05 |
| A92        | 4.0                | 10.5 | 60.7 | 0.1 | —   | 13.7    | 10.7 | —   | —   | 0.2  | 0.05 | 0.05 |
| A203       | 4.0                | —    | 71.6 | 1.1 | —   | 18.9    | 2.1  | 2.0 | —   | 0.2  | 0.05 | 0.05 |
| V197       | 3.9                | 7.1  | 64.6 | —   | 1.0 | 19.5    | —    | —   | 3.6 | 0.2  | 0.05 | 0.05 |
| V199       | 3.5                | 7.1  | 70.0 | —   | 0.9 | 16.5    | —    | —   | 3.6 | 0.25 | 0.10 | 0.05 |

35

Tests on the alloy V197 show its density to be 8.4 g/cc and a melting point in the region of 1300°C. Tables II, III and IV show respectively tensile, creep rupture and oxidation resistance properties. The weight losses of commercially available cast and wrought nickel-base alloys are included in Table IV for comparison.

Tests on the alloy V199 show its density to be 8.6 g/cc with a similar melting point to V197. Its tensile and creep/rupture properties are shown in Tables V and VI respectively.

TABLE II

| Test temperature °C | Tensile properties (V197)     |              |                                       |              |
|---------------------|-------------------------------|--------------|---------------------------------------|--------------|
|                     | Conventionally cast UTS (tsi) | % elongation | Unidirectionally solidified UTS (tsi) | % elongation |
| 20°C                | 50                            | 3            | 56                                    | 7            |
| 700°C               | 63                            | 3            | 71                                    | 8            |

TABLE III

| Test conditions | Creep rupture properties (V197) |              |                                       |              |
|-----------------|---------------------------------|--------------|---------------------------------------|--------------|
|                 | Conventionally cast Life (hr)   | % elongation | Unidirectionally solidified Life (hr) | % elongation |
| 19 tsi - 900°C  | —                               | —            | 37                                    | 27           |
| 8 tsi - 1000°C  | 17                              | 8            | 50                                    | 65           |
| 2 tsi - 1150°C  | 9                               | 5            | 44                                    | 50           |
| 6 tsi - 1000°C  | 70                              | 14           | —                                     | —            |

TABLE IV

| Material and condition                           | Oxidation resistance                                             |    |
|--------------------------------------------------|------------------------------------------------------------------|----|
|                                                  | Loss in weight<br>after 200 hr -<br>1250°C (mg/cm <sup>2</sup> ) |    |
| V197                                             | As cast                                                          | 3  |
|                                                  | Coated                                                           | 1  |
| Commercial cast nickel base                      |                                                                  | 5  |
| alloy - coated                                   |                                                                  |    |
| Commercial wrought nickel<br>base alloy - coated |                                                                  | 30 |

TABLE V

| Temper-<br>ature °C | Tensile properties (V199)      |                   |                     |                   |
|---------------------|--------------------------------|-------------------|---------------------|-------------------|
|                     | Unidirectionally<br>solidified |                   | Conventionally cast |                   |
|                     | UTS (tsi)                      | % elong-<br>ation | UTS (tsi)           | % elong-<br>ation |
| 20                  | 51                             | 8                 | 51                  | 11                |
| 700                 | 71                             | 5                 | 53                  | 2                 |

TABLE VI

| Test conditions | Creep rupture properties (V199) |              |                                |              |
|-----------------|---------------------------------|--------------|--------------------------------|--------------|
|                 | Conventionally cast             |              | Unidirectionally<br>solidified |              |
|                 | Life<br>(hr)                    | % elongation | Life<br>(hr)                   | % elongation |
| 4 tsi - 1100°C  | 8                               | 13           | 70                             | 30           |
| 2 tsi - 1150°C  | 10                              | 5            | 261                            | 30           |
| 6 tsi - 1000°C  | 70                              | 2            |                                |              |
| 15 tsi - 900°C  | 140                             | 2            |                                |              |

Tri-nickel aluminide exists only over a very narrow range in the Ni-Al phase diagram, and it is difficult to cast a component with a single phase structure. All the compositions according to the invention therefore are likely to contain, both in the conventionally cast condition and after unidirectional solidification, small quantities of nickel (gamma) and Ni-Al (beta) type phase, either separately or together. Metal carbides and borides are also likely to be present.

I claim:

45

1. An intermetallic compound material composed of in atomic percent, about 64.7 nickel, 3.7 chromium, 6.9 cobalt, 1.3 molybdenum, 17.2 aluminum, 5.9 titanium, 0.2 carbon, 0.05 boron, and 0.05 zirconium.
- 5 2. An intermetallic compound material composed of in atomic percent, about 64.2 nickel, 3.3 chromium, 7.1 cobalt, 0.8 molybdenum, 0.4 tungsten, 19.0 aluminum, 2.3 titanium, 1.3 niobium, 1.3 tantalum, 0.2 carbon, 0.05 boron, and 0.05 zirconium.
- 10 3. An intermetallic compound material composed of in atomic percent, about 62.8 nickel, 3.2 chromium, 7.3 cobalt, 0.7 molybdenum, 0.4 tungsten, 20.2 aluminum, 1.1 titanium, 2.1 niobium, 1.9 tantalum, 0.2 carbon, 0.05 boron, and 0.05 zirconium.
- 15 4. An intermetallic compound material composed of in atomic percent, about 64.5 nickel, 3.4 chromium, 7.2 cobalt, 0.7 molybdenum, 0.5 tungsten, 18.0 aluminum, 3.7 titanium, 0.8 niobium, 0.9 tantalum, 0.2 carbon, 0.05 boron, and 0.05 zirconium.
- 20 5. An intermetallic compound material composed of in atomic percent, about 61.5 nickel, 5.1 chromium, 7.9 cobalt, 1.8 tungsten, 19.9 aluminum, 3.5 tantalum, 0.2 carbon, 0.05 boron, and 0.05 zirconium.
6. An intermetallic compound material composed of
- 25 25 in atomic percent, about 62.9 nickel, 2.8 chromium, 6.5 cobalt, 1.0 molybdenum, 21.1 aluminum, 5.4 tantalum, 0.2 carbon, 0.05 boron, and 0.05 zirconium.
7. An intermetallic compound material composed of in atomic percent, about 64.8 nickel, 3.2 chromium,
- 30 30 6.8 cobalt, 1.1 molybdenum, 19.0 aluminum, 4.8 niobium, 0.2 carbon, 0.05 boron, and 0.05 zirconium.
8. An intermetallic compound material composed of in atomic percent, about 60.7 nickel, 4.0 chromium, 10.5 cobalt, 0.1 molybdenum, 13.7 aluminum, 10.7 titanium, 0.2 carbon, 0.05 boron, and 0.05 zirconium.
- 35 35 9. An intermetallic compound material composed of in atomic percent, about 71.6 nickel, 4.0 chromium, 1.1 molybdenum, 18.9 aluminum, 2.1 titanium, 2.0 niobium, 0.2 carbon, 0.05 boron, and 0.05 zirconium.
- 40 10. An intermetallic compound material composed of in atomic percent, about 64.6 nickel, 3.9 chromium, 7.1 cobalt, 1.0 tungsten, 19.5 aluminum, 3.6 tantalum, 0.2 carbon, 0.05 boron, and 0.05 zirconium.

\* \* \* \* \*

50

55

60

65